# EUROPEAN PATENT SPECIFICATION

(11) **EP 1 291 724 B1**
(45) Date of publication and mention of the grant of the patent: **14.12.2005**
(21) Application number: 02020082.0
(22) Date of filing: 06.09.2002
(51) Int. Cl.: G03G 5/06, G03G 5/047, G03G 5/043, G03G 5/082, G03G 15/04

(54) **Blue diode laser sensitive electrophotographic photoreceptor**
Elektrophotographischer Photoreceptor für blaues Laserlicht
Photorecepteur électrophotographique ayant une sensibilité à la lumière laser bleue

(30) Priority: 07.09.2001 US 947930
(43) Date of publication of application: 12.03.2003
(73) Proprietor: Xerox Corporation, Rochester, New York 14644 (US)
(72) Inventor: Parikh, Satish R., Rochester, New York 14625 (US); Carmichael, Kathleen M., Williamson, NY 14589 (US); Grabowski, Edward F., Webster, NY 14580 (US); Melnyk, Andrew R., Rochester, New York 14610 (US); Lin, Liang-Bih, Webster, New York 14580 (US); Ioannidis, Andronique, Webster, NY 14580 (US); Murti, Dasarao K., Mississauga, Ontario L5L 4T2 (CA); Hammond, Harold F., Webster, New York 14580 (US)
(74) Representative: Grünecker, Kinkeldey, Stockmair & Schwanhäusser Anwaltssozietät

(56) References cited:
- US-A- 4 927 726
- US-A- 5 849 445
- US-B1- 6 242 144

## Description

The present invention relates to imaging processes and printing machines. Specifically, the present invention is directed to the use of layered photoresponsive devices. More specifically, the present invention relates to the use of an improved layered photoresponsive device comprised generally of a transport layer and a photogenerating layer. The layered photoresponsive devices are useful as imaging members in various electrostatographic imaging systems, including those systems wherein electrostatic latent images are formed on the imaging member. Additionally, the photoresponsive devices can be selectively irradiated with blue light, for example, as generated by a known blue diode laser, to accomplish, for example, latent image formation by, for example, charged area development (CAD) or discharge area development (DAD) methodologies.

Numerous photoresponsive devices for electrostatographic imaging systems are known including selenium, selenium alloys, such as arsenic selenium alloys; layered inorganic photoresponsive, and layered organic devices. Examples of layered organic photoresponsive devices include those containing a charge transporting layer and a charge generating layer. Thus, for example, an illustrative layered organic photoresponsive device can be comprised of a conductive substrate, overcoated with a charge generator layer, which in turn is overcoated with a charge transport layer, and an optional overcoat layer overcoated on the charge transport layer. In a further "inverted" variation of this device, the charge transporter layer can be overcoated with the photogenerator layer or charge generator layer. Examples of generator layers that can be employed in these devices include, for example, charge generator materials such as selenium, cadmium sulfide, vanadyl phthalocyanine, x-metal free phthalocyanine, benzimidazole perylent (BZP), hydroxygallium phthalocyanine (HOGaPc), and trigonal selenium dispersed in binder resin, while examples of transport layers include dispersions of various diamines, reference for example, U.S. Patent No. 4,265,990.

U.S. Patent Nos. 6,242,144 and 4,927,726 disclose electrophotographic imaging members comprising, in the following sequence, a substrate, a charge-generating layer, and a charge-transport layer. The charge-generating layer of U.S. Patent No. 6,242,144 may contain trigonal selenium, metal-free phthalocyanine, or copper phthalocyanine; and the charge-transport layer may contain TAPC, TTA or mixtures thereof. The charge-generating layer disclosed in U.S. Patent No. 4,927,726 has a thickness ranging from 0.03 to 2 µm and may contain trigonal selenium, metal-free phthalocyanine, or vanadyl phthalocyanine; and the charge-transport layer has a thickness ranging from 2 to 100 µm and may contain TTA.

In the devices, imaging apparatuses, and processes of the prior art, various significant problems exist. For example, many conventional photoreceptor devices containing certain hole transport molecules (HTM) such as N,N'-diphenyl-N,N'-bis(3-methyl phenyl)-(1,1'-biphenyl)-4,4'-diamine (TPD) in an overlying charge transport layer cannot be successfully irradiated with specialized light sources, such as blue light generated from an aluminum-gallium-indium-nitride (AlGalnN) diode laser which source produces wavelength emissions, for example, of about 400 nanometers. This is because the certain hole transport molecules effectively absorb light at wavelengths below 420 nanometers and thus prevent incident light from reaching the underlying charge generator layer. The application of a blue light diode laser irradiation source to electrophotographic imaging systems could potentially offer a number of significant and economic advantages, such as higher image resolution, improved print quality, and lower energy consumption. These and other advantages are enabled with the apparatuses and processes of the present invention.

The present invention provides an imaging process comprising irradiating an imaging member with a diode laser at a wavelength of from 390 to 410 nanometers, said imaging member comprising a substrate, a charge generator layer having a thickness of from 0.01 to 5 µm (microns) overcoated on the substrate and being sensitive to blue light, and a charge transport layer having a thickness of from 5 to 50 µm (microns) overcoated on the charge generator layer and being transparent to blue light; developing the resulting latent image on the imaging member with a developer; and transferring the resulting developed image to a receiver member.

The present invention further provides a printing machine comprising an imaging member comprising a substrate, a charge generator layer having a thickness of from 0.01 to 5 µm (microns) overcoated on the substrate and being sensitive to blue light, and a charge transport layer having a thickness of from 5 to 50 µm (microns) overcoated on the charge generator layer and being transparent to blue light; a diode laser light source adapted to produce wavelengths of from 390 to 410 nanometers to irradiate the imaging member and form a latent image on the imaging member; a developer housing adapted to develop the latent image on the imaging member with a developer; a receiver member adapted to receive the resulting developed image; and an optional fixing member adapted to fix the resulting developed and transferred image to the receiver member.
Figure 1 illustrates the relative transparency of prototypical photoreceptor devices used in the present invention measured as a function of percentage transmission versus wavelength of exposed light.
Figure 2 illustrates the photo induced discharge curves (PIDC) measured at 670 and 400 nanometers of prototypical photoreceptor devices used in the present invention having a generator layer that includes hydroxygallium phthalocyanine or bisbenzimidazo(2,1-a-1',2'-b)anthra(2,1,9-def:6,5,10-d'e'f)diisoquinoline-6,11-dione and bisbenzimidazo(2,1-a:2',1'-a)anthra(2,1,9-def:6,5,10-d'e'f)diisoquinoline-10, 21-dione, (BZP) as a function of image potential versus exposure energy.
Figure 3 illustrates the photo induced discharge curve (PIDC) measured between 670 and 400 nanometers of prototypical photoreceptor devices used in the present invention having a generator layer that includes hydroxygallium phthalocyanine (HOGaPc) as a function of image potential versus exposure energy.
Figure 4 illustrates a cross section of an exemplary layered imaging article used in the present invention.
Figures 5 and 6 show the chemical structural formulas of hole transport molecules tritolylamine (TTA) and 1,1-bis (di-4-tolylaminophenyl) cyclohexane (TAPC), respectively.
Figure 7 shows the chemical structural formula of an exemplary coating resin for use in forming the coated layers used in the present invention.

The imaging members used in the present invention may be used to create blue sensitive imaging devices that allow the use of 400 nanometer blue laser diodes as an exposure source. High resolution laser printers require pointwise exposure using the smallest possible diameter laser beam. The minimum size of a laser beam is governed by the limits imposed by diffraction from the optical elements in the laser delivery system. The minimum beam size at the photoreceptor surface for a given set of optical elements is directly proportional to the wavelength of the laser illumination. The beam size for a 400 nanometer laser diode would be approximately half that observed with the same hardware and a 780 nanometer laser diode.

An advantage of the present invention is that the imaging process affords the following: higher resolution, higher print speed and a lower cost.

Preferred embodiments of the present invention are set forth in the sub-claims.

Further preferred is a charge transport layer containing a mixture of charge transport molecules 1,1-bis (di-4-tolylaminophenyl) cyclohexane (TAPC) and tritolyamine (TTA) in a relative weight ratio of from 0.1:1 to 1:0.1 and in a total amount of from 10 to 70 weight percent based on the total weight of the transport layer.

It is also preferred that the charge transport layer contains a mixture of charge transport molecules 1,1-bis (di-4-tolylaminophenyl) cyclohexane (TAPC) and TPD in a relative weight ratio of from 0.1:1 to 1:0.1 and in a total amount of from 10 to 70 weight percent based on the total weight of the transport layer.

In yet another preferred embodiment the charge generator layer contains a binder resin in an amount of from 50 to 99 weight percent based on the total weight of the charge generator layer.

In another preferred embodiment the charge generator layer contains a charge generator material of trigonal selenium ("t-Se") in an amount of from 1 to 25 weight percent based on the total weight of the charge generator layer.

Preferably the charge transport layer includes a binder resin.

It is more preferred that the charge transport layer binder resin is a polyester, a polycarbonate, a polyvinylbutaryl, a polyethercarbonate, an aryl amine polymer, a styrene copolymer in an amount of from 30 to 90 weight percent based on the total weight of the transport layer.

In embodiments the charge generating layer comprises photogenerating pigments.

In one embodiment the photogenerating pigments comprise selenium, cadmium sulfide, vanadyl phthalocyanine, x-metal free phthalocyanine, benzimidazole perylent (BZP), hydroxygallium phthalocyanine (HOGaPc), and trigonal selenium dispersed in binder resin.

Referring to the Figures, Figure 1 illustrates the relative transparency of prototypical photoreceptor transport layers measured as a function of percentage transmission versus wavelength in nanometers of the incident or exposed light. Curve 10 represents a control or baseline measure of transmission for a 75 micrometer thick polymeric ethylene terephthalate (PET) substrate which is a typical substrate used to fabricate photoreceptors. Curve 20 represents a measure of transmission for a device constructed with a 50/50 by weight mixture of m-TBD

N,N'-diphenyl-N,N'-bis(3-methyl phenyl)-(1,1'-biphenyl)-4,4'-diamine (TPD) and MAKROLON® polycarbonate as a free standing film. Curve 30 represents a measure of transmission for a device constructed with a 50/50 by weight mixture of 1,1-bis (di-4-tolylaminophenyl) cyclohexane (TAPC) hole transport molecule and MAKROLON® polycarbonate as a free standing film. Curve 40 represents a measure of transmission for a device constructed with a 50/50 by weight mixture of tritolyamine TTA hole transport molecule and MAKROLON® polycarbonate free standing film. Curve 50 represents a measure of transmission for a device constructed with a 50/50 by weight mixture of 1,1-bis (di-4-tolylaminophenyl) cyclohexane (TAPC) hole transport molecule and MAKROLON® polycarbonate as an air dried free standing film. Curve 60 represents a measure of transmission for a device constructed with a layer containing a 1:1 = TAPC: TPD mixture of hole transport molecules mixed 50/50 by weight with MAKROLON® polycarbonate as a free standing film.

Figure 2 illustrates the photo induced discharge curve (PIDC) measured at 400 nanometers of prototypical photoreceptor devices having a 670 and background generator layer (BGL) that includes BZP as a function of image potential in volts versus exposure energy in ergs per centimeters squared. Curve 100 represents the PIDC for the BZP control device at 400nm. Curve 110 represents the PIDC for the hydoxgallium phthalcyanine (HOGaPc). Curve 120 represents the PIDC for BZP at 400 nanometers. Curve 130 represents the PIDC for hydroxgallium phthalocyanine (HOGaPc) at 670 nanometers.

Figure 3 illustrates the photon induced discharge curves (PIDC) measured at 670 and 400 nanometers of prototypical photoreceptor devices having a background generator layer (BGL) that includes hydroxygallium phthalocyanine HOGaPc as a function of image potential in volts versus exposure energy in ergs per centimeters squared. Curve 200 represents the PIDC for the N,N'-diphenyl-N,N'-bis(3-methyl phenyl)-(1,1'-biphenyl)-4,4'-diamine (TPD) control device at 670nm and curve 230 represents the PIDC for the same device at 400nm. There is very little discharge at 400nm as the TPD containing device absorbs at this wavelength. Curve 220 represents the PIDC at 670nm for the device having a background generator layer (BGL) that includes HOGaPc and with 1,1-bis (di-4-tolylaminophenyl) cyclohexane (TAPC) as the hole transport molecule in the charge transport layer and appears to provide a PIDC with a comparable profile compared to curves 200 and 210. Curve 250 represents the PIDC of the TAPC device at 400nm and shows significant improvement in discharge over the TPD control device in curve 230. Curve 210 represents the PIDC for the device having a background generator layer (BGL) that includes HOGaPc and with a 1:1 by weight mixture of 1,1-bis (di-4-tolylaminophenyl) cyclohexane (TAPC) and N,N'-diphenyl-N,N'-bis(3-methyl phenyl)-(1,1'-biphenyl)-4,4'-diamine (TPD) hole transport molecules in the charge transport layer at 670nm and the PIDC is comparable to the control curve 200 and curve 220. Curve 240 represents the PIDC for the TPD/TAPC mixed device at 400NM. Note the intermediate discharge level between the pure TPD, curve 230, and pure TAPC, curve 250 at this same wavelength.

Figure 4 illustrates a cross section of an exemplary layered imaging article 40 including a substrate 50, a charge generator layer 60, a charge transport layer 70, and an optional overcoat layer 80, which article responds to as indicated in the above mentioned figures and as described herein when exposed to a suitable radiation source 90.

Figures 5 and 6 show the chemical structural formulas of tritolylamine (TTA) and 1,1-bis (di-4-tolylaminophenyl) cyclohexane (TAPC), respectively.

Figure 7 shows the chemical structural formula of an exemplary coating resin polycarbonate Z (PCZ), for use in forming the coated layers used in the present invention.

The present invention is particularly desirable for electrophotographic imaging layers which comprise two electrically operative layers, a charge generating layer and a charge transport layer.

The substrate may be opaque or substantially transparent and may comprise numerous suitable materials having the required mechanical properties. The substrate may further be provided with an electrically conductive surface. Accordingly, the substrate may comprise a layer of an electrically non-conductive or conductive material such as an inorganic or organic composition. As electrically non-conducting materials, there may be employed various resins known for this purpose including polyesters, polycarbonates, polyamides, and polyurethanes. The electrically insulating or conductive substrate may be flexible, semi-rigid, or rigid, and may have any number of different configurations such as, for example, a sheet, a scroll, an endless flexible belt, and a cylinder. The substrate may be in the form of an endless flexible belt which comprises a commercially available biaxially oriented polyester known as MYLAR™, MELINEX™, and KALADEX® available from E. I. du Pont de Nemours & Co.

The thickness of the substrate layer depends on numerous factors, including mechanical performance and economic considerations. The thickness of this layer may range from 65 micrometers to 150 micrometers, and preferably from 75 micrometers to 125 micrometers for optimum flexibility and minimum induced surface bending stress when cycled around small diameter rollers, for example, 19 millimeter diameter rollers. The substrate for a flexible belt may be of substantial thickness, for example, over 200 micrometers, or of minimum thickness, for example less than 50 micrometers, provided there are no adverse effects on the final photoconductive device. The surface of the substrate layer is preferably cleaned prior to coating to promote greater adhesion of the deposited coating composition. Cleaning may be effected by, for example, exposing the surface of the substrate layer to plasma discharge, or ion bombardment.

The electrically conductive ground plane may be an electrically conductive metal layer which may be formed, for example, on the coating article or substrate by any suitable coating technique, such as a vacuum depositing technique. Typical metals include aluminum, zirconium, niobium, tantalum, vanadium, hafnium, titanium, nickel, stainless steel, chromium, tungsten, molybdenum, and mixtures thereof. The conductive layer may vary in thickness over substantially wide ranges depending on the optical transparency and flexibility desired for the electrophotoconductive member. Accordingly, for a flexible photoresponsive imaging device, the thickness of the conductive layer may be from 20 Angstroms to 750 Angstroms, and more preferably from 50 Angstroms to 200 Angstroms for an optimum combination of electrical conductivity, flexibility and light transmission. Regardless of the technique employed to form the metal layer, a thin layer of metal oxide may form on the outer surface of most metals upon exposure to air. Thus, when other layers overlying the metal layer are characterized as "contiguous" layers, it is intended that these overlying contiguous layers may, in fact, contact a thin metal oxide layer that has formed on the outer surface of the oxidizable metal layer. Generally, for rear erase exposure, a conductive layer light transparency of at least 15 percent is desirable. The conductive layer need not be limited to metals. Other examples of conductive layers may be combinations of materials such as conductive indium tin oxide as a transparent layer for light having a wavelength between 4,000 Angstroms and 9,000 Angstroms or a conductive carbon black dispersed in a plastic binder as an opaque conductive layer.

After deposition of the electrically conductive ground plane layer, the blocking layer may be applied thereto. Electron blocking layers for positively charged photoreceptors allow holes from the imaging surface of the photoreceptor to migrate toward the conductive layer. For negatively charged photoreceptors, any suitable hole blocking layer capable of forming a barrier to prevent hole injection from the conductive layer to the opposite photoconductive layer may be utilized. The hole blocking layer may include polymers such as polyvinylbutyral, epoxy resins, polyesters, polysiloxanes, polyamides, or polyurethanes, or may be nitrogen containing siloxanes or nitrogen containing titanium compounds such as trimethoxysilyl propylene diamine, hydrolyzed trimethoxysilyl propyl ethylene diamine, N-beta-(aminoethyl) gamma-amino-propyl trimethoxy silane, isopropyl 4-aminobenzene sulfonyl, di(dodecylbenzene sulfonyl) titanate, isopropyl di(4-aminobenzoyl)isostearoyl titanate, isopropyl tri(N-ethylamino-ethylamino)titanate, isopropyl trianthranil titanate, isopropyl tri(N,N-dimethylethylamino)titanate, titanium-4-amino benzene sulfonate oxyacetate, titanium 4-aminobenzoate isostearate oxyacetate, [H₂N(CH₂)₄]CH₃Si(OCH₃)₂, gamma-aminobutyl) methyl diethoxysilane, and [H₂N(CH₂)₃]CH₃Si(OCH₃)₂, (gamma-aminopropyl)-methyl diethoxysilane, as disclosed in U.S. Patents 4,338,387, 4,286,033 and 4,291,110. Other suitable hole blocking layer polymer compositions are also described in U.S. Patent 5,244,762. These include vinyl hydroxyl ester and vinyl hydroxy amide polymers wherein the hydroxyl groups have been partially modified to benzoate and acetate esters which modified polymers are then blended with other unmodified vinyl hydroxy ester and amide unmodified polymers. An example of such a blend is a 30 mole percent benzoate ester of poly (2-hydroxyethyl methacrylate) blended with the parent polymer poly (2-hydroxyethyl methacrylate). Still other suitable hole blocking layer polymer compositions are described in U.S. Patent 4,988,597. These include polymers containing an alkyl acrylamidoglycolate alkyl ether repeat unit. An example of such an alkyl acrylamidoglycolate alkyl ether containing polymer is the copolymer poly(methyl acrylamidoglycolate methyl ether-co-2-hydroxyethyl methacrylate).

The blocking layer is continuous and may have a thickness of less than 10 micrometers because greater thicknesses may lead to undesirably high residual voltage. A hole blocking layer of between 0.005 micrometer and 1.5 micrometers is preferred because charge neutralization after the exposure step is facilitated and optimum electrical performance is achieved. The blocking layer may be applied by any suitable conventional technique such as spraying, dip coating, draw bar coating, gravure coating, silk screening, air knife coating, reverse roll coating, vacuum deposition, or chemical treatment. For convenience in obtaining thin layers, the blocking layer is preferably applied in the form of a dilute solution, with the solvent being removed after deposition of the coating by conventional techniques such as by vacuum, or heating. Generally, a weight ratio of blocking layer material and solvent of between 0.05:100 and 5:100 is satisfactory for spray coating.

Intermediate layers between the blocking layer and the adjacent charge generating or photogenerating layer may be desired to promote adhesion. For example, the adhesive layer may be employed. If such layers are utilized, they preferably have a dry thickness between 0.001 micrometer and 0.2 micrometer. Typical adhesive layers include film-forming polymers such as polyester, du Pont 49,000 resin, available from E. I. du Pont de Nemours & Co., VITEL-PE100™, available from Goodyear Rubber & Tire Co., polyvinylbutyral, polyvinylpyrrolidone, polyurethane, and polymethyl methacrylate.

The photoconductive layer may comprise any suitable photoconductive material well known in the art. Thus, the photoconductive layer may comprise, for example, a single layer of a homogeneous photoconductive material or photoconductive particles dispersed in a binder, or multiple layers such as a charge generating overcoated with a charge transport layer. The photoconductive layer may contain homogeneous, heterogeneous, inorganic or organic compositions. One example of an electrophotographic imaging layer containing a heterogeneous composition is described in U.S. Patent 3,121,006, wherein finely divided particles of a photoconductive inorganic compound are dispersed in an electrically insulating organic resin binder. Other well known electrophotographic imaging layers include amorphous selenium, halogen doped amorphous selenium, amorphous selenium alloys including selenium-arsenic, selenium-tellurium, selenium-arsenic-antimony, and halogen doped selenium alloys, and cadmium sulfide. Generally, these inorganic photoconductive materials are deposited as a relatively homogeneous layer.

Any suitable charge generating or photogenerating material may be employed as one of the two electrically operative layers in the multi-layer photoconductor embodiment. Typical charge generating materials include metal free phthalocyanine described in U.S. Patent 3,357,989, metal phthalocyanines such as copper phthalocyanine, vanadyl phthalocyanine, selenium containing materials such as trigonal selenium, bisazo compounds, quinacridones, substituted 2,4-diamino-triazines disclosed in U.S. Patent 3,442,781, and polynuclear aromatic quinones available from Allied Chemical Corporation under the tradename Indofast Double Scarlet, Indofast Violet Lake B, Indofast Brilliant Scarlet and Indofast Orange. Other examples of charge generating layers are disclosed in U.S. Patent Nos. 4,265,990, 4,233,384, 4,471,041, 4,489,143, 4,507,480, 4,306,008, 4,299,897, 4,232,102, 4,233,383, 4,415,639 and 4,439,507.

Any suitable inactive resin binder material may be employed in the charge generating layer. Typical organic resinous binders include polycarbonates, acrylate polymers, methacrylate polymers, vinyl polymers, cellulose polymers, polyesters, polysiloxanes, polyamides, polyurethanes, epoxies, and polyvinylacetals. Many organic resinous binders are disclosed, for example, in U.S. Patent Nos. 3,121,006 and 4,439,507. Organic resinous polymers may be block, random or alternating copolymers. The photogenerating composition or pigment can be present in the resinous binder composition in various amounts. When using an electrically inactive or insulating resin, it is preferred that there be high levels of particle-to-particle contact between the photoconductive particle population. This condition can be achieved, for example, with the photoconductive material present, for example, in an amount of at least 15 percent by volume of the binder layer with no limit on the maximum amount of photoconductor in the binder layer. If the matrix or binder comprises an active material, for example, poly-N-vinylcarbazole, the photoconductive material need only to comprise, for example, 1 percent or less by volume of the binder layer with no limitation on the maximum amount of photoconductor in the binder layer. Generally for charge generator layers containing an electrically active matrix or binder such as poly-N-vinyl carbazole or phenoxy-poly(hydroxyether), from 5 percent by volume to 60 percent by volume of the photogenerating pigment is dispersed in 40 percent by volume to 95 percent by volume of binder, and preferably from 7 percent to 30 percent by volume of the photogenerating pigment is dispersed in from 70 percent by volume to 93 percent by volume of the binder The specific proportions selected also depends to some extent on the thickness of the generating layer.

The thickness of the photogenerating binder layer is not particularly critical. Layer thicknesses from 0.05 micrometer to 40.0 micrometers may be satisfactory. The photogenerating binder layer containing photoconductive compositions and/or pigments, and the resinous binder material preferably ranges in thickness of from 0.1 micrometer to 5.0 micrometers, and has an optimum thickness of from 0.3 micrometer to 3 micrometers for best light absorption and improved dark decay stability and mechanical properties.

Other typical photoconductive layers include amorphous or alloys of selenium such as selenium-arsenic, selenium-tellurium-arsenic, or selenium-tellurium.

The active charge transport layer may comprise any suitable transparent organic polymer or non-polymeric material capable of supporting the injection of photo-generated holes and electrons from the charge generating layer and allowing the transport of these holes or electrons through the organic layer to selectively discharge the surface charge. The active charge transport layer not only serves to transport holes or electrons, but also protects the photoconductive layer from abrasion or chemical attack and therefore extends the operating life of the photoreceptor imaging member. The charge transport layer should exhibit negligible, if any, discharge when exposed to a wavelength of light useful in xerography, for example, 4,000 Angstroms to 8,000 Angstroms. Therefore, the charge transport layer is substantially transparent to radiation in a region in which the photoconductor is to be used. Thus, the active charge transport layer is a substantially non-photoconductive material which supports the injection of photogenerated holes or electrons from the generating layer. The active transport layer is normally transparent when exposure is effected through the active layer to ensure that most of the incident radiation is utilized by the underlying charge generating layer for efficient photogeneration. The charge transport layer in conjunction with the generating layer is a material which is an insulator to the extent that an electrostatic charge placed on the transport layer is not conductive in the absence of illumination, that is, does not discharge at a rate sufficient to prevent the formation and retention of an electrostatic latent image thereon.

An especially preferred transport layer employed in the electrically operative layer in the photoconductor embodiment comprises from 25 to 75 percent by weight of at least one charge transporting aromatic amine compound, and 75 to 25 percent by weight of a polymeric film forming resin in which the aromatic amine is soluble. Examples of charge transporting aromatic amines for charge transport layer(s) capable of supporting the injection of photogenerated holes of a charge generating layer and transporting the holes through the charge transport layer include 1,1-bis (di-4-tolylaminophenyl) cyclohexane (TAPC), and tritolyamine (TTA).

Any polymer which forms a solid solution with the hole transport molecule (HTM) is a suitable polymer material for use in forming a hole transport layer in a photoreceptor device. Any solvent which dissolves both the polymer and the HTM are suitable for use in fabricating photoreceptor devices. Any suitable inactive resin binder soluble in methylene chloride or other suitable solvent may be employed. Typical inactive resin binders soluble in methylene chloride include polycarbonate resin, polyvinylcarbazole, polyester, polyarylate, polystyrene, polyacrylate, polyether, and polysulfone. Molecular weights can vary from 20,000 to 1,500,000.

The preferred electrically inactive resin materials are polycarbonate resins have a molecular weight from 20,000 to 100,000, more preferably from 50,000 to 100,000. The materials most preferred as the electrically inactive resin material is poly(4,4'-dipropylidene-diphenylene carbonate) with a molecular weight of from 35,000 to 40,000, available as LEXAN 145™ from General Electric Company; poly(4,4'-isopropylidene-diphenylene carbonate) with a molecular weight of from 40,000 to 45,000, available as LEXAN 141 ™ from the General Electric Company; a polycarbonate resin having a molecular weight of from 50,000 to 100,000, available as MAKROLON™ from Farbenfabricken Bayer A.G., a polycarbonate resin having a molecular weight of from 20,000 to 50,000 available as MERLON™ from Mobay Chemical Company and poly(4,4'-diphenyl-1,1-cyclohexane carbonate). Methylene chloride solvent is a particularly desirable component of the charge transport layer coating mixture for adequate dissolving of all the components and for its low boiling point. However, the type of solvent selected depends on the specific resin binder utilized.

Any suitable and conventional technique may be utilized to apply the charge transport layer and the charge generating layer. Typical application techniques include spraying, dip coating, roll coating, and wire wound rod coating. Drying of the deposited coating may be effected by any suitable conventional technique such as oven drying, infra-red radiation drying, and air drying. Generally, the thickness of the transport layer is between 5 micrometers and 100 micrometers, but thicknesses outside this range can also be used. In general, the ratio of the thickness of the charge transport layer to the charge generating layer is preferably maintained from 2:1 to 200:1 and in some instances as great as 400:1.

The invention will further be illustrated in the following examples. Parts and percentages are by weight unless otherwise indicated.

### COMPARATIVE EXAMPLE I

A N,N'-diphenyl-N,N'-bis(3-methyl phenyl)-(1,1'-biphenyl)-4,4'-diamine (TPD) containing charge transport layer was formed on a hydroxygallium phthalocyanine (HOGaPc) containing charge generating layer device. The photo induced discharge curves (PIDC) for were measured at 670 and 400 nanometers and are shown in Figure 3.

### EXAMPLE II

A 1,1-bis (di-4-tolylaminophenyl) cyclohexane (TAPC) shown in Figure 5 containing charge transport layer was formed on both a BZP containing charge generating layer and a hydroxygallium phthalocyanine(HOGaPc) containing charge generating layer. The photoinduced discharge curves (PIDC) for the BZP and the HOGaPc devices were measured at 670 and 400nanometers and are shown in Figure 2. The hydroxygallium phthalocyanine device is discharged by both 670 nanometer and 400 nanometer light demonstrating that this device transmits 400 nanometer illumination to the generator layer. The BZP device discharges at 670 nanometers but does not discharge at 400 nanometers as the BZP pigment is not sensitive to 400 nanometer light. This demonstrates the need for a blue sensitive generation layer.

### EXAMPLE III

An N,N'-diphenyl-N,N'-bis(3-methyl phenyl)-(1,1'-biphenyl)-4,4'-diamine TPD:TAPC (1:1) containing charge transport layer was formed on a hydroxygallium phthalocyanine(HOGaPc) containing charge generating layer. The photoinduced discharge curves (PIDC) for the BZP and the HOGaPc devices were measured at 670 and 400 nanometers and are shown in Figure 3.

### EXAMPLE IV

### PHOTO-TRANSPARENCY AT 400 NANOMETERS

To assess the photo-transparency or photo-transmission of potential HTMs, four solutions were prepared with each solution containing a mixture of 50 weight percent of a HTM or mixture of two or more HTMs and 50 weight percent MAKROLON® 5705 polycarbonate together as 15 weight percent solids in methylene chloride. The four HTM or HTM combinations selected for analysis were: tritolyamine TTA; 1,1-bis (di-4-tolylaminophenyl) cyclohexane (TAPC); TAPC:TPD = 1:1; and N,N'-diphenyl-N,N'-bis(3-methyl phenyl)-(1,1'-biphenyl)-4,4'-diamine TPD. The solutions were coated to provide a film layer of 25 micrometers dry thickness on MYLAR® then dried at 125 °C for one minute. The films were removed from the MYLAR® substrate and the percent transmission was measured for the resulting free standing films and the results are illustrated graphically in Figure 1. Both tritolyamine TTA and 1,1-bis (di-4-tolylaminophenyl) cyclohexane (TAPC) transmit at 400 nanometers.

## Claims

1. An imaging process comprising:
irradiating an imaging member with a diode laser at a wavelength of from 390 to 410 nanometers, said imaging member comprising a substrate, a charge generator layer having a thickness of from 0.01 to 5 µm (microns) overcoated on the substrate and being sensitive to blue light, and a charge transport layer having a thickness of from 5 to 50 µm (microns) overcoated on the charge generator layer and being transparent to blue light;
developing the resulting latent image on the imaging member with a developer; and
transferring the resulting developed image to a receiver member.

2. A printing machine comprising:
an imaging member comprising a substrate, a charge generator layer having a thickness of from 0.01 to 5 µm (microns) overcoated on the substrate and being sensitive to blue light, and a charge transport layer having a thickness of from 5 to 50 µm (microns) overcoated on the charge generator layer and being transparent to blue light;
a diode laser light source adapted to produce wavelengths of from 390 to 410 nanometers to irradiate the imaging member and form a latent image on the imaging member;
a developer housing adapted to develop the latent image on the imaging member with a developer;
a receiver member adapted to receive the resulting developed image; and
an optional fixing member adapted to fix the resulting developed and transferred image to the receiver member.

3. The imaging process of claim 1 or the printing machine of claim 2, wherein the charge generator comprises metal free phthalocyanine, copper phthalocyanine, vanadyl phthalocyanine, hydroxygallium phthalocyanine, trigonal selenium, bisazo compounds, quinacridones substituted 2,4-diamino-triazines and/or polynuclear aromatic quinones.

4. The imaging process of claim 1 or the printing machine of claim 2, wherein the charge transport layer comprises a non-photoconductive material which supports the injection of photogenerated holes or electrons from the generating layer.

5. The imaging process of claim 1 or the printing machine of claim 2, wherein the charge transport layer contains the charge transport 1,1-bis (di-4-tolylaminophenyl) cyclohexane (TAPC) in an amount of from 10 to 70 weight percent based on the total weight of the transport layer.

6. The imaging process of claim 1 or the printing machine of claim 2, wherein the imaging member further comprises an overcoat layer being transparent to blue light of from 390 to 430 nanometers.

7. The imaging process of claim 1 or the printing machine of claim 2, wherein the blue light transparent transport layer contains charge transport molecules of 1,1-bis (di-4-tolylaminophenyl) cyclohexane (TAPC), tritolyamine (TTA) or mixtures thereof, and the blue light sensitive generator layer contains trigonal selenium.

## Patentansprüche

1. Ein bildgebendes Verfahren, das:
das Bestrahlen eines bildgebenden Bauteils mit einem Diodenlaser bei einer Wellenlänge von 390 bis 410 Nanometern, wobei das bildgebende Bauteil ein Trägermaterial, eine ladungserzeugende Schicht mit einer Dicke von 0,01 bis 5 µm (Mikron), die auf das Trägermaterial aufgetragen und gegenüber blauem Licht empfindlich ist, und eine ladungstransportierende Schicht mit einer Dicke von 5 bis 50 µm (Mikron), die auf die ladungserzeugende Schicht aufgetragen und gegenüber blauem Licht transparent ist, umfasst;
das Entwickeln des resultierenden, latenten Bildes auf dem bildgebenden Bauteil mit einem Entwickler; und
das Übertragen des resultierenden, entwickelten Bildes auf ein aufnehmendes Bauteil umfasst.

2. Eine Druckmaschine, umfassend:
ein bildgebendes Bauteil, das ein Trägermaterial, eine ladungserzeugende Schicht mit einer Dicke von 0,01 bis 5 µm (Mikron), die auf das Trägermaterial aufgetragen und gegenüber blauem Licht empfindlich ist, und eine ladungstransportierende Schicht mit einer Dicke von 5 bis 50 µm (Mikron), die auf die ladungserzeugende Schicht aufgetragen und gegenüber blauem Licht transparent ist, umfasst;
eine Diodenlaser-Lichtquelle, die dahingehend angepasst ist, Wellenlängen von 390 bis 410 Nanometern zu erzeugen, um das bildgebende Bauteil zu bestrahlen und auf dem bildgebenden Bauteil ein latentes Bild auszubilden;
ein Entwicklergehäuse, das dahingehend angepasst ist, das latente Bild auf dem bildgebenden Bauteil mit einem Entwickler zu entwickeln;
ein aufnehmendes Bauteil, das dahingehend angepasst ist, das resultierende, entwickelte Bild zu empfangen; und
ein optionales fixierendes Bauteil, das dahingehend angepasst ist, das resultierende, entwickelte und auf das aufnehmende Bauteil transferierte Bild zu fixieren.

3. Das bildgebende Verfahren von Anspruch 1 oder die Druckmaschine von Anspruch 2, worin der Ladungserzeuger Metall-freies Phthalocyanin, Kupferphthalocyanin, Vanadylphthalocyanin, Hydroxygalliumphthalocyanin, trigonales Selen, Bisazo-Verbindungen, Chinacridone, substituierte 2,4-Diaminotriazine und/oder mehrkernige aromatische Chinone umfasst.

4. Das bildgebende Verfahren von Anspruch 1 oder die Druckmaschine von Anspruch 2, worin die ladungstransportierende Schicht ein nicht-photoleitfähiges Material umfasst, das die Injektion von lichtgenerierten Löchern oder Elektronen aus der erzeugenden Schicht unterstützt.

5. Das bildgebende Verfahren von Anspruch 1 oder die Druckmaschine von Anspruch 2, worin die ladungstransportierende Schicht das ladungstransportierende Molekül 1,1-Bis(di-4-tolylaminophenyl)cyclohexan (TAPC) in einer Menge von 10 bis 70 Gewichtsprozent, bezogen auf das gesamte Gewicht der transportierenden Schicht, enthält.

6. Das bildgebende Verfahren von Anspruch 1 oder die Druckmaschine von Anspruch 2, worin das bildgebende Bauteil zusätzlich eine Überzugsschicht enthält, die gegenüber blauem Licht von 390 bis 430 Nanometern transparent ist.

7. Das bildgebende Verfahren von Anspruch 1 oder die Druckmaschine von Anspruch 2, worin die gegenüber blauem Licht transparente Transportschicht die ladungstransportierenden Moleküle 1,1-Bis (di-4-tolylaminophenyl) cyclohexan (TAPC), Tritolylamin (TTA) oder Mischungen davon enthält und worin die gegenüber blauem Licht empfindliche, erzeugende Schicht trigonales Selen enthält.

## Revendications

1. Procédé de formation d'image comprenant les étapes consistant à :
irradier un élément de formation d'image avec une diode laser à une longueur d'onde de 390 à 410 nanomètres, ledit élément de formation d'image comprenant un substrat, une couche de génération de charge présentant une épaisseur de 0, 01 à 5 µm (micromètres) déposée de manière à recouvrir le substrat et sensible à la lumière bleue, et une couche de transport de charge présentant une épaisseur de 5 à 50 µm (micromètres) déposée de manière à recouvrir la couche de génération de charge et transparente à la lumière bleue ;
développer l'image latente résultante sur l'élément de formation d'image avec un rêvélateux ; et
transférer l'image développée résultante à un élément récepteur.

2. Appareil d'impression comprenant :
un élément de formation d'image comprenant un substrat, une couche de génération de charge présentant une épaisseur de 0,01 à 5 µm (micromètres) déposée de manière à recouvrir le substrat et sensible à la lumière bleue, et une couche de transport de charge présentant une épaisseur de 5 à 50 µm (micromètres) déposée de manière à recouvrir la couche de génération de charge et transparente à la lumière bleue ;
une source de lumière laser diode capable de produire des longueurs d'onde de 390 à 410 nanomètres pour irradier l'élément de formation d'image et former une image latente sur l'élément de formation d'image;
une boite de révélateur capable de développer l'image latente sur l'élément de formation d'image avec un révélateur ;
un élément récepteur capable de recevoir l'image développée résultante ; et
un élément de fixage facultatif capable de fixer l'image développée et transférée résultante sur l'élément récepteur.

3. Procédé de formation d'image selon la revendication 1 ou appareil d'impression selon la revendication 2, dans lequel le générateur de charge comprend de la phtalocyanine exempte de métal, de la phtalocyanine de cuivre, de la vanadylphtalocyanine, de l'hydroxygalliumphtalocyanine, du sélénium trigonal, des composés bisazonïques, des 2,4-diaminotriazines substituées par des quinacridones et/ou des quinones aromatiques polynucléaires.

4. Procédé de formation d'image selon la revendication 1 ou appareil d'impression selon la revendication 2, dans lequel la couche de transport de charge comprend un matériau non photoconducteur qui supporte l'injection d'électrons ou de trous photogénérés de la couche de génération.

5. Procédé de formation d'image selon la revendication 1 ou appareil d'impression selon la revendication 2, dans lequel la couche de transport de charge contient le transporteur de charge 1,1-bis (di-4-tolylaminophényl) cyclohexane (TAPC) en une quantité de 10 à 70 % en poids par rapport au poids total de la couche de transport.

6. Procédé de formation d'image selon la revendication 1 ou appareil d'impression selon la revendication 2, dans lequel l'élément de formation d'image comprend en outre une couche le recouvrant transparente à la lumière bleue de 390 à 430 nanomètres.

7. Procédé de formation d'image selon la revendication 1 ou appareil d'impression selon la revendication 2, dans lequel la couche de transport transparente à la lumière bleue contient des molécules de transport de charge de 1,1 -bis (di-4-tolylaminophényl)cyclohexane (TAPC), de tritolylamine (TTA) ou des mélanges de celles-ci, et la couche de génération sensible à la lumière bleue contient du sélénium trigonal.
